

# United States Patent [19]

Kopatz et al.

[11] Patent Number: 4,802,915

[45] Date of Patent: Feb. 7, 1989

[54] PROCESS FOR PRODUCING FINELY DIVIDED SPHERICAL METAL POWDERS CONTAINING AN IRON GROUP METAL AND A READILY OXIDIZABLE METAL

4,687,510 8/1987 Cheney et al. .... 75/0.5 BA  
4,687,511 8/1987 Paliwal et al. .... 75/05. BA  
4,723,993 2/1988 Kopatz et al. .... 75/0.5 C  
4,731,110 3/1988 Kopatz et al. .... 75/0.5 BA

[75] Inventors: Nelson E. Kopatz, Sayre; Joseph E. Ritsko; Walter A. Johnson, both of Towanda, all of Pa.

Primary Examiner—Wayland Stallard  
Attorney, Agent, or Firm—Donald R. Castle

[73] Assignee: GTE Products Corporation, Stamford, Conn.

## [57] ABSTRACT

[21] Appl. No.: 185,713

Alloys of a first group of metals containing at least one iron group metal and one or more easily oxidizable metals can be formed by forming an aqueous solution of the first group of metals, forming solids containing the metals from the solution, reducing the solids to a metallic powder, converting the metallic powder to metallic alloy spherical powders, agglomeration the spherical powder with one or more easily oxidizable metals in a non-oxidizing atmosphere, thereafter the agglomerates are subjected to a sufficient temperatures under non-oxidizing conditions to form an alloy. Alternatively, the easily oxidizable metals can be agglomerated with the solids containing the iron group metal prior to converting the agglomerates to a spherical alloy powder.

[22] Filed: Apr. 25, 1988

[51] Int. Cl.<sup>4</sup> ..... B22F 9/24

[52] U.S. Cl. ..... 75/0.5 AA; 75/0.5 BA;  
75/0.5 AC; 75/0.5 BC

[58] Field of Search ..... 75/0.5 AA, 0.5 BA, 0.5 BC,  
75/0.5 AC

## [56] References Cited

### U.S. PATENT DOCUMENTS

3,652,259 3/1972 Knopp ..... 75/0.5 BA  
4,348,224 9/1982 Gingerich et al. ..... 75/0.5 AA  
4,397,682 8/1983 Watanabe et al. ..... 75/0.5 BA  
4,613,371 9/1986 Cheney et al. ..... 75/0.5 C

16 Claims, No Drawings

**PROCESS FOR PRODUCING FINELY DIVIDED SPHERICAL METAL POWDERS CONTAINING AN IRON GROUP METAL AND A READILY OXIDIZABLE METAL**

**FIELD OF THE INVENTION**

This invention relates to the preparation of metal powders containing an iron group metal and a readily oxidizable metal and to iron group based metal alloy powders containing such readily oxidizable metals. More particularly it relates to the production of such powders having substantially spherical particles.

**BACKGROUND OF THE INVENTION**

Metal alloy powders heretofore have been produced by gas or water atomization of molten ingots of the alloy. It has not been generally practical to produce the metal alloy powders directly from the individual metal powders because of the difficulty in obtaining uniformity of distribution of the metals. It is difficult to obtain certain powders containing readily oxidizable metals such as aluminum because of the tendency of those metals to form the respective oxides which are stable during processing.

U.S. Pat. No. 3,909,241 relates to free flowing powders which are produced by feeding agglomerates through a high temperature plasma reactor to cause at least partial melting of the particles and collecting the particles in a cooling chamber containing a protective gaseous atmosphere where the particles are solidified. In this patent the powders are used for plasma coating and the agglomerated raw materials are produced from slurries of metal powders and binders. Both U.S. Pat. Nos. 3,663,667 and 3,909,241 are assigned to the same assignee as the present invention.

In U.S. Pat. No. 4,613,371, issued Sept. 23, 1986, also assigned to the assignee of this invention, there is disclosed a process for making ultra-fine powder by directing a stream of molten droplets at a repellent surface whereby the droplets are broken up and repelled and thereafter solidified as described therein. While there is a tendency for spherical particles to be formed after rebounding, it is stated that the molten portion may form elliptical shaped or elongated particles with rounded ends.

U.S. Pat. Nos. 3,663,667; 3,909,241; 3,974,245; 4,502,885 and 4,508,788, all relate to formation of free flowing powders via the production of agglomerates and feeding agglomerates through a high temperature plasma reactor to cause at least partial melting of the particles. Resulting powders are spherical and free flowing. These patents relate to the use of metal agglomerates and not to powder particles which necessarily have a uniform distribution of constituents throughout the agglomerate.

It is believed therefore that a relatively simple process which enables finely divided iron group metal or iron group based alloy powders containing such readily oxidizable metals to be produced from sources of the individual metals would be an advancement in the art.

**SUMMARY OF THE INVENTION**

In accordance with one aspect of this invention there is provided a process comprising:

(a) forming an aqueous solution containing at least one metal from the iron group metal,

(b) forming from said solution a reducible solid material selected from salts of the iron group metal, oxides of said iron group metal, hydroxides of said iron group metal and mixtures thereof,

5 (c) reducing this solid material to form metallic powder particles,

(d) combining such metallic powder particles with finely divided particles of at least one easily oxidizable metal in a non-oxidizing atmosphere to form agglomerates therefrom and,

10 (e) subjecting the agglomerates to a sufficient temperature in a non-oxidizing atmosphere to form an alloy.

In accordance with another aspect of this invention there is provided a process comprising:

15 (a) forming an aqueous solution containing at least one metal from the iron group metal,

(b) forming a reducible solid material selected from salts of said iron group metal, oxides of said iron group metal, hydroxides of said iron group metal and mixtures thereof from the aqueous solution,

(c) reducing such solid material to form metallic powder particles,

(d) entraining at least a portion of these powder particle in a carrier gas,

25 (e) feeding the entrained particles and the carrier gas into a high temperature zone and maintaining the particles in the zone for a sufficient time to melt at least about 50% by weight of the particles and to form droplets therefrom and

30 (f) cooling such droplets to form metal particles having essentially a spherical shape,

(g) combining the spherical shaped particles with finely divided particles of at least one easily oxidizable metal in a non-oxidizing atmosphere to form an agglomerate and,

35 (h) subjecting said agglomerates to a sufficient temperature in a non-oxidizing atmosphere to form an alloy.

In preferred embodiments of both aspects the alloy is formed using a plasma.

**DETAILS OF THE PREFERRED EMBODIMENTS**

For a better understanding of the present invention, 45 together with other and further objects, advantages, and capabilities thereof, reference is made to the following disclosure and appended claims in connection with the foregoing description of some of the aspects of the invention.

50 While it is preferred to use metal powders as starting materials in the practice of this invention because such materials dissolve more readily than other forms of metals, however, use of the metallic powders is not essential. Metallic salts that are soluble in water or in an aqueous mineral acid can be used. When alloys are desired, the metallic ratio of the various metals in the subsequently formed solids of the salts, oxides or hydroxides can be calculated based upon the raw material input or the solid can be sampled and analyzed for the metal ratio in the case of alloys being produced. The metal values can be dissolved in any water soluble acid. The acids can include the mineral acids as well as the organic acids such as acetic, formic and the like. Hydrochloric is especially preferred because of cost and availability.

55 After the metal sources are dissolved in the aqueous acid solution, the resulting solution can be subjected to sufficient heat to evaporate water. The metal com-

pounds, for example, the oxides, hydroxides, sulfates, nitrates, chlorides, and the like, will precipitate from the solution under certain pH conditions. The solid materials can be separated from the resulting aqueous phase or the evaporation can be continued. Continued evaporation results in forming particles of a residue consisting of the metallic compounds. In some instances, when the evaporation is done in air, the metal compounds may be the hydroxides, oxides or mixtures of the mineral acid salts of the metals and the metal hydroxides or oxides. The residue may be agglomerated and contain oversized particles. The average particle size of the materials can be reduced in size, generally below about 20 micrometers by milling, grinding or by other conventional methods of particle size reduction.

After the particles are reduced to the desired size they are heated in a reducing atmosphere at a temperature above the reducing temperature of the salts but below the melting point of the metals in the particles. The temperature is sufficient to evolve any water of hydration and the anion. If hydrochloric acid is used and there is water of hydration present the resulting wet hydrochloric acid evolution is very corrosive thus appropriate materials of construction must be used. The temperatures employed are below the melting point of any of the metals therein but sufficiently high to reduce and leave only the cation portion of the original molecule. In most instances a temperature of at least about 500° C. is required to reduce the compounds. Temperatures below about 500° C. can cause insufficient reduction while temperatures above the melting point of the metal result in large fused agglomerates. If more than one metal is present the metals in the resulting multi-metal particles can either be combined as intermetallics or as solid solutions of the various metal components. In any event there is a homogenous distribution throughout each particle of each of the metals. The particles are generally irregular in shape. If agglomeration has occurred during the reduction step, particle size reduction by conventional milling, grinding and the like can be done to achieve a desired average particle size for example less than about 20 micrometers with at least 50% being below about 20 micrometers.

In preparing the powders of the present invention, a high velocity stream of at least partially molten metal droplets is formed. Such a stream may be formed by any thermal spraying technique such as combustion spraying and plasma spraying. Individual particles can be completely melted (which is the preferred process), however, in some instances surface melting sufficient to enable the subsequent formation of spherical particles from such partially melted particles is satisfactory. Typically, the velocity of the droplets is greater than about 100 meters per second, more typically greater than 250 meters per second. Velocities on the order of 900 meters per second or greater may be achieved under certain conditions which favor these speeds which may include spraying in a vacuum.

In the preferred process of the present invention, a powder is fed through a thermal spray apparatus. Feed powder is entrained in a carrier gas and then fed through a high temperature reactor. The temperature in the reactor is preferably above the melting point of the highest melting component of the metal powder and even more preferably considerably above the melting point of the highest melting component of the material to enable a melting during relatively short residence time in the reaction zone.

The stream of dispersed entrained molten metal droplets may be produced by plasma-jet torch or gun apparatus of conventional nature. In general, a source of metal powder is connected to a source of propellant gas. 5 A means is provided to mix the gas with the powder and propel the gas with entrained powder through a conduit communicating with a nozzle passage of the plasma spray apparatus. In the arc type apparatus, the entrained powder may be fed into a vortex chamber which communicates with and is coaxial with the nozzle passage which is bored centrally through the nozzle. In an arc type plasma apparatus, an electric arc is maintained between an interior wall of the nozzle passage and an electrode present in the passage. The electrode has a 10 diameter smaller than the nozzle passage with which it is coaxial to so that the gas is discharged from the nozzle in the form of a plasma jet. The current source is normally a DC source adapted to deliver very large currents at relatively low voltages. By adjusting the magnitude of the arc powder and the rate of gas flow, torch temperatures can range from 5500 degrees centigrade up to about 15,000 degrees centigrade. The apparatus generally must be adjusted in accordance with the melting point of the powders being sprayed and the gas employed. In general, the electrode may be retracted within the nozzle when lower melting powders are utilized with an inert gas such as nitrogen while the electrode may be more fully extended within the nozzle when higher melting powders are utilized with an inert gas such as argon.

In the induction type plasma spray apparatus, metal powder entrained in an inert gas is passed at a high velocity through a strong magnetic field so as to cause a voltage to be generated in the gas stream. The current source is adapted to deliver very high currents, on the order of 10,000 amperes, although the voltage may be relatively low such as 10 volts. Such currents are required to generate a very strong direct magnetic field and create a plasma. Such plasma devices may include 35 additional means for aiding in the initiation of a plasma generation, a cooling means for the torch in the form of annular chamber around the nozzle.

In the plasma process, a gas which is ionized in the torch regains its heat of ionization on exiting the nozzle 45 to create a highly intense flame. In general, the flow of gas through the plasma spray apparatus is effected at speeds at least approaching the speed of sound. The typical torch comprises a conduit means having a convergent portion which converges in a downstream direction to a throat. The convergent portion communicates with an adjacent outlet opening so that the discharge of plasma is effected out the outlet opening.

Other types of torches may be used such as an oxy-acetylene type having high pressure fuel gas flowing 55 through the nozzle. The powder may be introduced into the gas by an aspirating effect. The fuel is ignited at the nozzle outlet to provide a high temperature flame.

Preferably the powders utilized for the torch should be uniform in size and composition. A relatively narrow size distribution is desirable because, under set flame conditions, the largest particles may not melt completely, and the smallest particles may be heated to the vaporization point. Incomplete melting is a detriment to the product uniformity, whereas vaporization and decomposition decreases process efficiency. Typically, the size ranges for plasma feed powders of this invention are such that 80 percent of the particles fall within about a 15 micrometer diameter range.

The stream of entrained molten metal droplets which issues from the nozzle tends to expand outwardly so that the density of the droplets in the stream decreases as the distance from the nozzle increases. Prior to impacting a surface, the stream typically passes through a gaseous atmosphere which solidifies and decreases the velocity of the droplets. As the atmosphere approaches a vacuum, the cooling and velocity loss is diminished. It is desirable that the nozzle be positioned sufficiently distant from any surface so that the droplets remain in a droplet form during cooling and solidification. If the nozzle is too close, the droplets may solidify after impact.

The stream of molten particles may be directed into a cooling fluid. The cooling fluid is typically disposed in a chamber which has an inlet to replenish the cooling fluid which is volatilized and heated by the molten particles and plasma gases. The fluid may be provided in liquid form and volatilized to the gaseous state during the rapid solidification process. The outlet is preferably in the form of a pressure relief valve. The vented gas may be pumped to a collection tank and reliquified for reuse.

The choice of the particle cooling fluid depends on the desired results. If large cooling capacity is needed, it may be desirable to provide a cooling fluid having a high thermal capacity. An inert cooling fluid which is non-flammable and non-reactive may be desirable if contamination of the product is a problem. In other cases, a reactive atmosphere may be desirable to modify the powder. Argon and nitrogen are preferable non-reactive cooling fluids. Hydrogen may be preferable in certain cases to reduce oxides and protect the powder from unwanted reactions. Liquid nitrogen may enhance nitride formation. If oxide formation is desired, air, under selective oxidizing conditions, is a suitable cooling fluid.

Since the melting plasmas are formed from many of the same gases, the melting system and cooling fluid may be selected to be compatible.

The cooling rate depends on the thermal conductivity of the cooling fluid and the molten particles to be cooled, the size of the stream to be cooled, the size of individual droplets, particle velocity and the temperature difference between the droplet and the cooling fluid. The cooling rate of the droplets is controlled by adjusting the above mentioned variables. The rate of cooling can be altered by adjusting the distance of the plasma from the liquid bath surface. The closer the nozzle to the surface of the bath, the more rapidly cooled the droplets.

Powder collection is conveniently accomplished by removing the collected powder from the bottom of the collection chamber. The cooling fluid may be evaporated or retained if desired to provide protection against oxidation or unwanted reactions.

The particle size of the spherical powders will be largely dependent upon the size of the feed into the high temperature reactor. Some densification occurs and the surface area is reduced thus the apparent particle size is reduced. The Preferred form of particle size measurement is by micromerograph, sedigraph or Microtrac. A majority of the particles will be below about 20 micrometers or finer. The desired size will depend upon the use of the alloy. For example, in certain instances such as microcircuitry applications extremely finely divided materials are desired such as less than about 3 micrometers.

The powdered materials of this invention are essentially spherical particles which are essentially free of elliptical shaped material and essentially free of elongated particles having rounded ends, is shown in European patent application No. W08402864.

Spherical particles have an advantage over non-spherical particles in injection molding and pressing and sintering operations. The lower surface area of spherical particles as opposed to non-spherical particles of comparable size, makes spherical particles easier to mix with binders and easier to dewax.

To further illustrate this invention, the following non-limiting examples are presented. All parts, proportions and percentages are by weight unless otherwise indicated.

#### EXAMPLE 1

About 650 parts of iron powder and about 350 parts of cobalt powder are dissolved in about 4000 parts of 10 N HCl using a glass lined agitated reactor.

Ammonium hydroxide is added to a pH of about 6.5-7.5. The iron and cobalt are precipitated as an intimate mixture of hydroxides. This mixture is then evaporated to dryness. The mixture is then heated to about 350° C. in air for about 3 hours to remove the excess ammonium chloride. This mixture is then hammer-milled to produce a powder having greater than 50% of the particles smaller than about 50 micrometers with no particles larger than about 100 micrometers. These milled particles are heated in a reducing atmosphere of H<sub>2</sub> at a temperature of about 700° C. for about 3 hours. Finely divided particles containing 65% iron and 35% cobalt are formed.

The iron-cobalt powder particles are entrained in an argon carrier gas. The particles are fed to a Metco 9MB plasma gun at a rate of about 10 pounds per hour. The gas is fed at the rate of about 6 cubic feet per hour. The plasma gas (Ar+H<sub>2</sub>) is fed at the rate of about 70 cubic feet per hour. The torch power is about 11 KW at about 40 55 volts and 200 amperes. The molten droplets exit into a chamber containing inert gas. The resulting powder contains two fractions, the major fraction consists of the spherical shaped resolidified particles. The minor fraction consists of particles having surfaces which have been partially melted and resolidified.

The resulting powder after air classifying to achieve an average size below about 20 micrometers is mixed with a binder and finely divided aluminum powder. A polyvinylbutyral polymer is dissolved in alcohol. The mixture of the iron-cobalt powder and the aluminum powder is dispersed in the alcohol-polymer solution to form a slurry. This slurry is then pumped to a closed cycle, nitrogen atmosphere spray dryer. Uniform agglomerates of Fe, Co and Al are produced. These agglomerates are then heated to about 500°-600° C. in an H<sub>2</sub> atmosphere to remove the PVB binder.

The Fe-Co-Al agglomerates are entrained in an argon carrier gas. The particles are fed to a Metco 9MB plasma gun at a rate of about 10 pounds per hour. The gas is fed at the rate of about 6 cubic feet per hour. The plasma gas (Ar+H<sub>2</sub>) is fed at the rate of about 70 cubic feet per hour. The torch power is about 27.5 KW at about 50 volts and 550 amperes. The molten droplets exit into a chamber containing inert gas. The resulting powder contains two fractions, the major fraction consists of the spherical shaped resolidified particles.

The minor fraction consists of particles having surfaces which have been partially melted and resolidified.

## EXAMPLE 2

About 650 parts of iron powder and about 350 parts of cobalt powder are dissolved in about 4000 parts of 10 N HCl using a glass lined agitated reactor.

Ammonium hydroxide is added to a pH of about 6.5-7.5. The iron and cobalt are precipitated as an intimate mixture of hydroxides. This mixture is then evaporated to dryness. The mixture is then heated to about 350° C. in air for about 3 hours to remove the excess ammonium chloride. This mixture is then hammer-milled to produce a powder having greater than 50% of the particles smaller than about 50 micrometers with no particles larger than about 100 micrometers. These milled particles are heated in a reducing atmosphere of 15 H<sub>2</sub> at a temperature of about 700° C. for about 3 hours. Finely divided particles containing 65% iron and 35% cobalt are formed.

The resulting powder after air classifying to achieve an average size below about 20 micrometers is mixed with a binder and finely divided aluminum powder. A polyvinylbutyral polymer is dissolved in alcohol. The mixture of the iron-cobalt powder and the aluminum powder is dispersed in the alcohol-polymer solution to form a slurry. This slurry is then pumped to a closed cycle, nitrogen atmosphere spray dryer. Uniform agglomerates of Fe, Co and Al are produced. These agglomerates are then heated to about 500°-600° C. in an H<sub>2</sub> atmosphere to remove the PVB binder.

The Fe-Co-Al agglomerates are entrained in an argon carrier gas. The particles are fed to a Metco 9MB plasma gun at a rate of about 10 pounds per hour. The gas is fed at the rate of about 6 cubic feet per hour. The plasma gas (Ar+H<sub>2</sub>) is fed at the rate of about 70 cubic feet per hour. The torch power is about 27.5 KW at about 50 volts and 550 amperes. The molten droplets exit into a chamber containing inert gas. The resulting powder contains two fractions, the major fraction consists of the spherical shaped resolidified particles.

The minor fraction consists of particles having surfaces which have been partially melted and resolidified.

While there has been shown and described what are considered the preferred embodiments of the invention, it will be obvious to those skilled in the art that various changes and modifications may be made therein without departing from the scope of the invention as defined by the appended claims.

What is claimed:

1. A process comprising:

- (a) forming an aqueous solution containing at least one metal from the iron group metal,
- (b) forming from said solution a reducible solid material selected from salts of said iron group metal, oxides of said iron group metal, hydroxides of said iron group metal and mixtures thereof,
- (c) reducing said material to form metallic powder particles,
- (d) entraining at least a portion of said powder particle in a carrier gas,
- (e) feeding said entrained particles and said carrier gas into a high temperature zone and maintaining said particles in said zone for a sufficient time to melt at least about 50% by weight of said particles, and to form droplets therefrom and
- (f) cooling said droplets to form metal particles having essentially a spherical shape,
- (g) combining said spherical shaped particles with finely divided particles of at least one easily oxidiz-

able metal in a non-oxidizing atmosphere to form an agglomerate and,

(h) subjecting said agglomerates to a sufficient temperature in a non-oxidizing atmosphere to form an alloy.

5 2. A process according to claim 1 wherein said mineral acid is selected from the group consisting of hydrochloric, sulfuric and nitric acids.

3. A process according to claim 2 wherein said mineral acid is hydrochloric acid.

4. A process according to claim 1 wherein said alloying is achieved by entraining said agglomerates in a carrier gas and feeding said agglomerates and said gas into a high temperature zone for a time sufficient to form metallic alloy particles having essentially a spherical shape.

5 5. A process according to claim 1 wherein said agglomerates are formed by utilizing a binder and spray drying and then the binder is removed from said agglomerates.

6. A process according to claim 4 wherein said metals in said first group are selected from the iron group metals.

7. A process according to claim 5 wherein said metals from said first group are iron and cobalt and the metal from said second group is aluminum.

8. A process according to claim 4 wherein said high temperature zone is created by a plasma touch.

9. A process comprising:

- (a) forming an aqueous solution containing at least one metal from the iron group metal,
- (b) forming from said solution a reducible solid material selected from salts of said iron group metal, oxides of said iron group metal, hydroxides of said iron group metal and mixtures thereof,
- (c) reducing said material to form metallic powder particles,
- (d) combining said metallic powder particles with finely divided particles of at least one easily oxidizable metal in a non-oxidizing atmosphere to form agglomerates therefrom and,
- (e) subjecting said agglomerates to a sufficient temperature in a non-oxidizing atmosphere to form an alloy.

10. A process according to claim 9 wherein said mineral acid is selected from the group consisting of hydrochloric, sulfuric and nitric acids.

11. A process according to claim 10 wherein said mineral acid is hydrochloric acid.

12. A process according to claim 9 wherein said alloying is achieved by entraining said agglomerates in a carrier gas and feeding said agglomerates and said gas into a high temperature zone for a time sufficient to form metallic alloy particles having essentially a spherical shape.

13. A process according to claim 9 wherein said agglomerates are formed by utilizing a binder and spray drying and then the binder is removed from said agglomerates.

14. A process according to claim 12 wherein said metals in said first group are selected from the iron group metals.

15. A process according to claim 13 wherein said metals from said first group are iron and cobalt and the metal from said second group is aluminum.

16. A process according to claim 12 wherein said high temperature zone is created by a plasma touch.

\* \* \* \* \*